

Jan. 15, 1935.

F. M. CLARK

1,988,299

OIL FOR TRANSFORMERS AND THE LIKE

Filed April 23, 1932



Inventor:  
Frank M. Clark,  
by *Charles V. Tully*  
His Attorney.

## UNITED STATES PATENT OFFICE

1,988,299

## OIL FOR TRANSFORMERS AND THE LIKE

Frank M. Clark, Pittsfield, Mass., assignor to  
General Electric Company, a corporation of  
New York

Application April 23, 1932, Serial No. 607,142

5 Claims. (Cl. 252—1)

The present invention relates to the suppression of sludge formation in petroleum products, such as the oil content of electrical devices, such as transformers, wherein mineral oil is used for 5 cooling and insulating purposes.

A semi-solid precipitate known as sludge is formed in mineral oil during transformer service when such oil is heated without special precautions to an elevated temperature. The operating temperatures of the oil vary with the character and loading of transformers but ordinarily they are well below 150° C., as observed at the hottest point in a transformer. Sludge, when formed, clogs the cooling ducts and lowers 10 the dielectric qualities of the oil. It consists largely of tarry or asphaltic polymerization and esterification products. Although sludged transformer oil may be reclaimed by the use of acid or fuller's earth, or both, and used over again 15 when mixed with new oil, the net effect of the sludging of transformer oil is an economic loss and a constant threat to the continued safe operation of the apparatus.

While it is possible to employ in a transformer, or the like, a highly refined mineral oil in which sludge will not be formed under operating conditions, such oil not only is expensive but it has been found to be subject to an even more objectionable acid formation. In the highly refined oil, which has been freed of unsaturated hydrocarbons, corrosive acids of the acetic acid type are formed. These attack actively metal parts of the device, and seriously affect the mechanical and electrical properties of the insulation immersed therein.

In some respects an unrefined oil distillate, that is, a chosen fraction of crude oil distillation, is better suited for dielectric purposes than a highly refined oil. Its market price is only about a tenth the price of highly refined oil. However, it has been found that the sludge forming characteristics of such oil may vary from shipment to shipment. Its use thus entails a serious laboratory control expense. In any event, as elsewhere more fully explained the unrefined distillate forms sludge more readily than a refined oil. Therefore, it has been the practice to employ for transformer purposes a special partially refined oil in which a compromise is

made between various qualities including sludging and acid formation.

Partially refined oil, that is, hydrocarbon distillates from which unsaturated components have been partially removed (by treatment with ordinary sulphuric acid as distinguished from the fuming sulphuric acid employed for producing a highly refined oil) costs about one-half as much as highly refined oil.

As a result of a long series of experiments I have discovered that when there is associated with unrefined oil a small amount of a naphthyl amine compound, ordinarily less than one per cent by weight, that sludging is substantially suppressed. In accordance with my invention 10 sludging is not only suppressed but the advantages of the low cost unrefined distillate are secured without difficulties from the excessive acid formation characterizing the highly refined product.

The accompanying drawing, Fig. 1, is a side elevation of a transformer which is shown as being illustrative of the most useful commercial application of my invention; and Fig. 2 is a graph showing by accelerated sludging tests the 15 beneficial effect of my invention on mineral oil.

The beneficial effect of such amine in the oil appears to be due to both a retardation of the polymerization and esterification reactions whereby sludge products are formed and a peptizing effect whereby such products as may be formed by such action are kept in solution and hence do not interfere with the function of the oil in the transformer or the like.

The benefits of my invention also may be obtained to a substantial extent with partly refined hydrocarbon oils which may be employed in combination with such naphthyl amine for a period of service which is much longer than the service life of partly refined oil unassociated 20 with such amine.

In carrying out my invention a primary or secondary naphthyl amine, such for example as alpha or beta naphthyl amine, in desired amount is dissolved in a convenient quantity of hydrocarbon oil which then is added to the main body of oil in which suppression of sludging is desired. I prefer to employ phenyl alpha naphthyl amine. I prefer to add to the oil about one-half of one per cent by weight of the amine. I 25 30 35 40 45 50

prefer also to employ unrefined distillates having a flash point not less than 125 to 130° C. and a viscosity of approximately 50 to 60 seconds Saybolt Universal at 37.8° C. Unrefined distillates 5 may have iodine values as high as 18 to 20. Partially refined oil, such as commonly used in transformers has iodine values of about 7 to 8. Highly refined oil has a zero iodine value. I prefer to use an oil having an iodine value not 10 higher than 15 to 18, no free sulphur, less than 5/10 per cent fixed sulphur; although as high as 3/4% may be used.

One example of a suitable distillate has the following properties:

|    |                                                |            |
|----|------------------------------------------------|------------|
| 15 | Flash point                                    | 135° C.    |
|    | Burn point                                     | 150° C.    |
|    | Specific gravity 15.5°                         | .900       |
|    | Viscosity 37.8°                                | 58 seconds |
| 20 | Inorg. content                                 | 0          |
|    | Acidity less than 1.0 mg. NaOH per gram of oil |            |
|    | Iodine number                                  | 18         |
|    | Fixed sulphur                                  | .5 percent |
|    | Free sulphur                                   | 0          |

25 Referring to Fig. 1 of the drawing, the transformer which is illustrated comprises a tank 1, containing an iron core 2, and electrical windings 3, the terminals of which are indicated at 4, 4'. The core and windings are immersed in oil 30 as indicated at 5. As indicated by legend on the drawing the oil 5 contains dissolved therein a naphthyl amine.

35 The benefits of my invention have been demonstrated under service conditions. In my tests the effect of a great many different materials on such oil has been investigated. As an oil-filled type transformer contains a large quantity of oil and as sludge may require several years to make its appearance in a transformer 40 which operates at a temperature only moderately above ambient temperatures, it would require a long time ordinarily to test the efficacy of a material as an anti-sludging reagent in mineral oil under service conditions but tests 45 have been devised whereby the formation of sludge in oil mixes is accelerated. In accordance with one such test small oil samples (and any substance associated therewith) are heated at 110° C. in contact with copper (which accelerates sludging) and then such sludge as may be formed is centrifugally separated from the oil in suitable test tubes. Its volume may be observed. In accordance with an even more rapid test small samples of oil are subjected at a temperature of 140° C. in a closed container (bomb) 50 for 24 hours to the effect of pure oxygen at a pressure of 250 pounds to the square inch. The sludge formed under these conditions is centrifugally separated and observed. It is usually 55 expressed in percent by comparison with weight of the original oil sample.

60 In Fig. 2 I have shown graphically the result of a series of tests made with mineral oil containing phenyl alpha naphthyl amine which was subjected to normal operating conditions in a transformer containing over four hundred gallons of oil. The results obtained were found to check with preliminary tests. They were checked again with bomb tests involving treatment with oxygen under pressure as described above, and again the results were found to be in agreement.

65 Referring to Fig. 2, the length of time oil samples were subjected to accelerated sludging 70 conditions are plotted as abscissæ in days of 75

hours each. The percent of sludge formation noted after centrifuging are plotted as ordinates. Curve "a" shows the results obtained with oil samples which were the same as the oil which was introduced into a transformer, namely ordinary transformer oil which had been partly refined by ordinary sulphuric acid and to which was added by weight about 1/16 percent of phenyl alpha naphthyl amine. After forty days of heating at 110° C. in contact with copper only 10 1% of sludge could be observed in a test sample as indicated by curve "a". Curve "b" shows the effect of a similar test on similar oil samples taken from the transformer after three months' 15 service. One percent of sludge could be observed after thirty-five days heating of the sample. Curve "c" shows the results obtained with small samples taken from the transformer after six months' service. One percent of sludge appears in a sample after about thirty days' 20 heating. Curve "d" shows that thereafter little change took place as after one year's service only slightly more sludge could be noted in a test sample heated for thirty days. Curve "e" shows check tests performed on new commercial transformer oil (unassociated with naphthyl amine or other retarder). About one percent of sludge 25 appeared in such new oil after twenty-five days' heating under the same conditions. Curve "f" shows the result of the same accelerated sludge 30 test on an unrefined distillate. This curve rises very steeply and shows 1.2 percent of sludge in a test sample in twelve to thirteen days. Unrefined distillate containing a naphthyl amine shows itself by test to be substantially equal to 35 a partially refined transformer oil (curve "e") or even better in some cases. No separate curve for such a combination has been shown as it tends nearly to coincide with other curves and would thus tend to confuse the graph.

40 Bomb test experiments as above described have not been plotted but led to the same conclusion. New transformer oil containing 1/2% phenyl alpha naphthyl amine gave .05% sludge by weight. After three months' service the 45 weight of sludge obtained by bomb test was unchanged. After six months' service .06% of sludge was observed in a test sample. After one year's service .05% of sludge was observed. In a sample of new transformer oil .06% of sludge 50 was observed by this test. Similar favorable results have been observed with other naphthyl amines. These results are all the more surprising because of the fact that some amines have been found to be accelerators of sludging.

55 What I claim as new and desire to secure by Letters Patent of the United States is:

1. A petroleum composition suitable for use at an elevated temperature comprising potentially sludging mineral oil and a quantity of naphthyl amine associated therewith, said oil so modified being resistant for a materially longer time to the formation of sludge at elevated temperature than similar oil which is unassociated with such amine.

60 2. A petroleum composition comprising potentially sludging mineral oil and phenyl alpha naphthyl amine associated therewith, said oil so modified being resistant for a materially longer time to the formation of sludge at elevated temperature than when unassociated with such amine.

65 3. A composition suitable for use as an insulating and cooling dielectric material in electric devices comprising mineral oil having an 70

iodine value within the limits of about 7 to 20 and tending by itself when heated during service to form insoluble, semi-solid products, and about one-half of one per cent of phenyl alpha naphthyl amine, whereby the formation of such semi-solid products is materially retarded.

4. The process of preventing sludging in mineral oil containing sludge-forming constituents which comprises maintaining a naphthyl

amine in association with such oil during use under conditions which in the absence of such amine would form sludge therein.

5. A composition comprising the combination of an unrefined mineral oil and about one-half of one per cent by weight thereof of phenyl alpha naphthylamine.

FRANK M. CLARK.